

# United States Patent Office

2,842,319

Patented July 8, 1958

1

2,842,319

## METHOD OF PRODUCING ULTRA-CLEAN COAL

Wilhelm Reerink, Essen-Bredeney, Walter Müschenborn,  
Essen, and Erich Nötzold, Essen-Haarzopf, Germany

No Drawing. Application October 21, 1953  
Serial No. 387,538

Claims priority, application Germany November 5, 1952

17 Claims. (Cl. 241—14)

The invention relates to a method of producing ultra-clean coal by wet cleaning.

All of the known methods to produce ultra-clean coal by wet processes have the disadvantage that the yield of such ultra-clean coal, i. e., of coal having ash content considerably less than 0.5%, is rather small resulting in a correspondingly low economy of these methods. This disadvantage is also present in the conventional flotation process carried out with repeated treatment of the concentrates which may be subjected to comminution between the successive steps.

In contrast to the known wet methods, ultra-clean coal concentrates with an ash content substantially below 0.5% are produced by the process according to the invention, whereby these concentrates are obtained in a considerable yield.

The new process is based on the discovery that the ultra-clean constituents to be separated from the coal, namely the pure vitrain components, and possibly clarains with low spore content, have a substantially lower mechanical strength than the coal constituents having a higher ash content, i. e. the mineral constituents and the coal constituents rendered impure by impregnation.

According to the basic principle of the invention, the new process is carried out as follows:

The coal to be treated, i. e. either a fine disintegrated coal or, preferably, a suitable bed coal (lump coal) after being properly comminuted is classified to a suitable fine material size, whereupon the fine material from this classification is subjected to flotation. Thereafter the concentrate of this preliminary flotation is classified or screened again by means of a finer mesh screen, the oversize grains from this classification are further comminuted and are subjected either together with the undersize grains from this classification, or separately therefrom, to one or several further flotation steps.

In this process the coarser grain fraction from the screening step preceding the preliminary flotation, on the one hand, and the oversize grain fraction from the subsequent screening step, i. e. the constituents which primarily contain the mineral impregnated stronger grain, on the other hand, are separated by mere mechanical means and always the finest material containing the purest constituents is subjected to flotation, which may be repeated several times, if need.

According to the present invention, the new process includes steps of selectively comminuting the starting coal material according to the different mechanical strengths of its petrographic constituents. Thus, with lump coal as a starting material, the preliminary comminution is preferably not carried out in such a manner that a grain size required for the flotation, is obtained, said grain size being generally about .75 mm., i. e. the grinding apparatus used is adjusted to a substantially coarser grain size. In this case the harder fractions having a higher ash content remain in coarser condition than the more brittle particles which are more easily crushed, the latter being mainly

2

vitrain particles of low ash content, than the mass of the refuse. In this process, the constituents obtained from veins having high durain and spore contents or from mineralized fractions are separated in the first screening step or sink directly in the preliminary flotation if they reach it.

In the preliminary flotation, the operation is preferably carried out in such a manner that independently of the grain size of the material treated a positive separation between the purest particles raised into the concentrate and the impure grains to be rejected is obtained by adjusting the flotation range to approximately .75 mm., if need to 1 mm. The oversize grain from the preliminary comminution, the size of which is above the selected flotation limit and which contains the main portion of the ash, can either be rejected at the outset or may be subjected to another comminution by recycling it, while continuously separating the grain above a grain size found to be suitable, such as 3 mm. to avoid undesirably high losses of pure coal in the oversize grain. The grain between 1 and 3 mm. is further comminuted and the fraction below 1 mm. of said comminuted material is subjected to flotation.

The comminution of the intermediate grain may be carried out separately by means of selective grinding, the limit between the oversize grain to be rejected and the fine material to be subjected to flotation being successively lowered in each of the successive grinding steps.

The comminution should be conducted in such a manner so as to obtain a highly uniform grain distribution having a low percentage of very fine grain and a high output of gritty coarser grain.

The impurities from the material obtained in this comminution step are separated by means of a flotation step carried out in a very satisfactory manner, because the selective separation takes place under the action of the higher weight of the harder, coarser and less buoyant fractions. Less effective flotation media are advantageously employed in this operation, because the then resulting foam concentrates can subsequently be easily purified.

The concentrates from the preliminary flotation may be subjected to one or more after-flotations if necessary. These concentrates represent a relatively coarse-grained product having an ash content in the range between 0.8 to 1% which, in addition to ultra-clean particles of finest grain, generally contains extremely fine, highly dispersed mineral and very fine fusain splinters having a high ash content, and in addition to these ordinary ash carriers, coarser particles having a high vitrain content coalesced with ash-containing particles or mineralized impregnated particles.

The comminution and subsequent screening of this concentrate should be carried out to obtain a grain size of at least  $100\mu$ , and if possible even below that size. Of course, this depends upon the nature of the coal in its raw state, though not to such extent that particles of the refuse freed from vitrain particles are unnecessarily split up, which would be disadvantageous to the further flotation.

The intermediate comminution may be effected in a baffle-plate mill or in grinding mills or the like. This is followed by a screening step to separate the oversize grain, for example above  $100\mu$ , said grain having also a higher ash content. This screening step, according to an important feature of the present invention, is carried out in a novel manner under addition of large amounts of water by means of screen centrifuges with finely calibrated slots, slits or holes. This is particularly advantageous in case the extremely fine material separated thereby is immediately subjected to a further flotation, which has to

be carried out with very little solid pulp content due to the fineness of the material particles.

The oversize grain remaining in the centrifuge can either be recycled to the mill or returned to the preliminary flotation, or it may be entirely discarded. Preferably, the oversize grain is subjected to a further flotation because it mostly contains a fraction of coarse vitrain particles freed by the comminution. This justifies the further flotation from an economical point of view.

According to another modification of the process according to this invention, the centrifugal treatment may precede the comminution, i. e. it may take place immediately after the first flotation, whereupon only the coarse concentrate of the centrifuge is fed to the mill. As compared with the first embodiment of the invention, this modified process has the advantage that not the entire amount of the very fine grain and of the water contained in the foam has to be passed through the mill. Only the coarse grain, i. e. in a considerably thickened condition, is fed to the mill. This is usually more favorable for operating the mill.

The flotation foam is destroyed to a great extent during centrifuging.

In the example just described, the coarse grain of the centrifuge is subjected to the very fine comminution and the comminuted material is fed either to the same or to a separate flotation apparatus, treating only the latter material, to separate the freed impurities. The material may be returned to the screening centrifuge if desired.

Furthermore, it may be advantageous to treat the material which has been repeatedly ground in a separate centrifuge to avoid unfavorable repeated very fine grinding of the impurities. The coarse grain of this centrifuge is either discarded or returned to the preliminary flotation.

Finally, the extremely finely ground refined material is subjected to a final flotation, likewise with multiple repetition of the concentrates, whereby the latter are yielded with an ash content in the order of 0.3% and lower, which heretofore could not be obtained by purely mechanical means.

During the individual flotation steps, the pH values which were ascertained as the most favorable are preferably adjusted.

The wastes of the last flotation constitute a concentrate having a very low ash content of usually only 1 to 3% of ash, which has commercial usefulness.

All of the coal-containing wastes of the process are preferably separated by treating them with oil-containing substances for the purpose of phase reversal and simultaneous dispersion in water, followed by separation of the dispersing agent containing the fine wastes from the coal in a centrifuge so as to obtain pure wastes and ordinary commercial coal.

According to a further development of the new process, products can be obtained which have properties particularly suitable for special purposes. In this case, components which are adapted to acquire such qualities by being mixed with one another, for example concentrates composed of baking and nonbaking coals, are separately prepared and then mixed, whereby the components are preferably mixed prior to the dewatering step, and the mixture containing these components is filtered or advantageously centrifuged, resulting in an extremely intimate mixture.

It is also possible to first prepare a suitable mixture from the respective types of coal and then to subject the same to the treatment according to the new process.

If in such cases there is any risk that the mixture might disintegrate, it is recommended to first subject the components separately to preliminary flotation and to bring them together in the course of the intermediate comminution, so that in the subsequent flotation the components are treated together in the mixture. During this step, there is no danger that the mixture may disintegrate.

Such operations do not result in an enlargement of the flotation apparatus, since the amount of material passing through the flotation in any case requires a certain number of cells.

In order to impart to the prepared concentrates certain properties desired for their special purpose or use, they will be subjected, for example, to a coking treatment or low temperature carbonization, and hydrocarbons, such as pitches, oils, tars, or the like may be added to these concentrates. Such operation is carried out in a suitable apparatus in which the material is exposed to pressures and/or vacuum resulting displacement of the water layers from the surfaces of the coal particles by the hydrocarbons, whereby the latter become intimately bonded to the coal particles. The particles thus hydrophobized can be dewatered in a very satisfactory manner in screen-type centrifuges, whereby no coal particles will pass into the filtrate water, i. e. any particles of refuse dispersed in the water will pass through the screens. As a result of this, the ashes are removed to a still greater extent.

Ultra-clean coal mixed with pitches in this way can be coked in a superior manner, even if the coal itself is not cokable.

In this case it may be to further advantage to briquet the material prior to the coking step, such briquetting operation being readily carried out with coal concentrates treated with hydrocarbons, because these coal concentrates can be compressed into very strong briquettes without previous drying. These briquettes, when coked, result in extremely homogeneous bodies having excellent properties.

A numerical example of the results obtained with the new process is given below:

35

*Example*

|    | Steps.                                       | Fraction, percent | Ash, percent                |
|----|----------------------------------------------|-------------------|-----------------------------|
| 1  | Starting coal.....                           | 100               | 8.5.                        |
|    | Oversize grain, 5-3 mm.....                  | 3                 | 50, waste.                  |
| 2  | Oversize grain, 3-1 mm.....                  | 5                 | 20, after-comminution.      |
|    | Very fine grain, 1-0 mm.....                 | 92                | 6.5.                        |
| 3  | Material subjected to flotation, 1-0 mm..... | 97                | 7.2.                        |
|    | Refined coal.....                            | 74                | 0.8, very fine comminution. |
|    | Wastes.....                                  | 23                | 28, phase reversal.         |
| 4  | Ultra-clean coal.....                        | 52                | 0.3.                        |
|    | Wastes 2.....                                | 22                | 2 or 2nd concentrate.       |
|    | Total wastes.....                            | 23+22=45          | 15.2, phase reversal.       |
| 50 | Oil coal.....                                | 40                | 7.                          |
|    | Pure wastes.....                             | 5                 | 81.                         |

This invention is obviously subject to considerable modification and hence we do not choose to be limited to the examples disclosed herein but rather to the scope of the appended claims.

We claim:

1. A method of producing ultra-clean coal having a very low ash content comprising in combination the steps of selectively comminuting a starting coal according to the different mechanical strengths of its petrographic constituents, screening said comminuted material by means of a first screen, subjecting the fine material from said screening step to a preliminary flotation, screening the concentrate from said preliminary flotation step by means of a second screen of finer mesh than said first screen, further breaking-up the oversize grain from said finer mesh screening step, subjecting the undersize grain from said finer mesh screening step and said further broken-up oversize grain from said finer mesh screening step to a further flotation and collecting the concentrate from said further flotation step.

2. A method of producing ultra-clean coal having a very low ash content comprising in combination the steps of selectively comminuting a starting coal according to the different mechanical strengths of its petrographic con-

stituents, screening said comminuted material by means of a first screen, subjecting the fine material from said screening step to a preliminary flotation, screening the concentrate from said preliminary flotation step by means of a second screen of finer mesh than said first screen, further breaking-up the oversize grain from said finer mesh screening step, subjecting the undersize grain from said finer mesh screening step and said further broken-up oversize grain from said finer mesh screening step jointly to a further flotation and collecting the concentrate from said further flotation step.

3. A method of producing ultra-clean coal having a very low ash content comprising in combination the steps of selectively comminuting a starting coal according to the different mechanical strengths of its petrographic constituents, screening said comminuted material by means of a first screen, subjecting the fine material from said screening step to a preliminary flotation, screening the concentrate from said preliminary flotation step by means of a second screen of finer mesh than said first screen, further breaking up the oversize grain from said finer mesh screening, subjecting the undersize grain of said finer mesh screening step and said further broken-up oversize grain from said finer mesh screening step separately to further flotation and collecting the concentrate from said further flotation steps.

4. A method of producing ultra-clean coal having a very low ash content comprising in combination the steps of selectively comminuting a starting coal according to the different mechanical strengths of its petrographic constituents, screening said comminuted material by means of a first screen, subjecting the fine material from said screening step to a preliminary flotation, subjecting the concentrate from said preliminary flotation step to a further breaking-up operation, screening said latter broken-up concentrate by means of a second screen of finer mesh than said first screen, further breaking-up the oversize grain from said finer mesh screening step, subjecting the undersize grain of said finer mesh screening step and said further broken-up oversize grain from said finer mesh screening step to a further flotation and collecting the concentrate from said further flotation step.

5. A method of producing ultra-clean coal having a very low ash content comprising in combination the steps of selectively comminuting a starting coal according to the different mechanical strengths of its petrographic constituents, screening said comminuted material by means of a first screen, subjecting the fine material from said screening step to a preliminary flotation, screening the concentrate from said preliminary flotation step by means of a second screen of finer mesh than said first screen, further breaking-up the oversize grain from said finer mesh screening step, subjecting the undersize grain from said finer mesh screening step to a further flotation, further screening said further broken-up oversize grain from said finer mesh screening step, subjecting the undersize grain from said further screening step to a further flotation and collecting the concentrates from said further flotation steps.

6. A method of producing ultra-clean coal having a very low ash content according to claim 1 characterized by very finely comminuting the coarser grain from said first screening step of the comminuted starting coal and subjecting the comminuted material to the same treatment as the finer grain after the first screening step.

7. A method of producing an ultra-clean coal having a very low ash content according to claim 1 characterized by subjecting the oversize grain from said first screening step of the comminuted starting coal to the same flotation treatment as the undersize grain.

8. A method of producing ultra-clean coal having a very low ash content according to claim 5 characterized by subjecting the oversize grain from said further screening step to the same flotation treatment as the undersize grain.

9. A method of producing ultra-clean coal having a very low ash content according to claim 5 characterized by subjecting the oversize grain from said second screening step to independent screening and subjecting the oversize grain separated thereby to flotation treatment.

10. A method of producing ultra-clean coal having a very low ash content comprising in combination the steps of screening a fine coal produced by selective decomposition into components of different strengths, subjecting the fine material from screening step to a preliminary flotation, screening the concentrate from said preliminary flotation step by means of a second screen of finer mesh than said first screen, further breaking-up the oversize grain from said finer mesh screening step, subjecting the undersize grain from said finer mesh screening step, and further broken-up oversize grain from said finer mesh screening step to a further flotation and collecting the concentrate from said further flotation step.

11. The method of producing ultra-clean coal having a very low ash content comprising in combination the steps of selectively comminuting a starting coal according to the different mechanical strengths of its petrographic constituents, screening said comminuted material by means of a first screen, subjecting the fine material from said screening step to a preliminary flotation, centrifugally sifting the concentrate from said preliminary flotation step, further comminuting the oversize grain from said centrifugal sifting step, subjecting the undersize grain from said centrifugal sifting step and said further comminuted oversize grain from said centrifugal sifting step to a further flotation and collecting the concentrate from said further flotation step.

12. A method of producing ultra-clean coal having a very low ash content according to claim 1 characterized by oil-wetting said oversize grain with simultaneous dispersion in water, and mechanically separating the oil-wetted mass.

13. A method of producing ultra-clean coal having a very low ash content comprising in combination the steps of selectively comminuting a mixture of different types of coal selected in accordance with the required properties of the ultra-clean coal concentrates to be produced, screening said comminuted material by means of a first screen, subjecting the fine material from said screening step to a preliminary flotation, screening the concentrate from said preliminary flotation step by means of a second screen of finer mesh than said first screen, further breaking-up the oversize grain from said finer mesh screening step, subjecting the undersize grain from said finer mesh screening step and said further broken-up oversize grain to a further flotation and collecting the concentrate from said further flotation step.

14. A method of producing ultra-clean coal having a very low ash content according to claim 5 characterized by mixing said concentrates and subsequently dewatering them.

15. A method of producing ultra-clean coal having a very low ash content according to claim 5 characterized by mixing the concentrate from said preliminary flotation step with said further comminuted oversize grain and subjecting the mixture to after-flotation.

16. A method of producing ultra-clean coal having a very low ash content according to claim 1 characterized by adding to said coal concentrate substances adapted to influence the properties of said concentrate.

17. A method of producing ultra-clean coal having a very low ash content according to claim 1 characterized by wetting said concentrate with a hydrocarbon, displacing the water envelope from the material particles, and dewatering the hydrophobised concentrate.

## References Cited in the file of this patent

## UNITED STATES PATENTS

|           |          |               |
|-----------|----------|---------------|
| 143,745   | Bradford | Oct. 21, 1873 |
| 1,258,869 | Callow   | Mar. 12, 1918 |
| 1,854,659 | Lehmann  | Apr. 19, 1932 |
| 2,136,074 | Crawford | Nov. 8, 1938  |
| 2,376,703 | Kuhlwein | May 22, 1945  |

## OTHER REFERENCES

United States Bureau of Mines Information Circular 7481, October 1945, "Methods of Producing Ultra-clean Coal for Electrode Carbon in Germany," 13 pages.